

# United States Patent Office

2,805,945

Patented Sept. 10, 1957

## 1

2,805,945

### MAINSpring COMPOSED OF NICKEL BASE ALLOYS

Reinhard Straumann, Waldenburg, Switzerland

No Drawing. Application March 29, 1954,  
Serial No. 419,579

Claims priority, application Switzerland January 28, 1949

7 Claims. (Cl. 75—171)

The present invention is a continuation-in-part application of my copending application Serial No. 267,694, filed on January 22, 1952 (and abandoned since the filing of the present application).

The present invention relates to a new corrosion-resistant, substantially non-magnetic highly elastic mainspring for watches.

Many kinds of alloys have already been proposed for use as springs in watches. Thus U. S. Patent No. 2,072,489 is directed to a nickel iron alloy with a hardening addition of beryllium, for the springs of thermo-compensated oscillating systems, for example balance springs for clocks and watches, in which with a content of 25—40% of nickel and 0.5—2% of beryllium with a calculated quantity of alloying addition of at least one of the metals of the group consisting of molybdenum, chromium and tungsten amounting to a total content of 5—12%, 0.5—2% of titanium is also alloyed, with the object that in addition to the great hardness achieved and the low temperature coefficient, the dependence of the latter and its secondary error on the fixing temperature is greatly reduced to the rate of 0.5—1 second for each degree centigrade variation of the fixing temperature. This alloy containing as main constituent iron is well suited for the production of hairsprings or balance springs, but—in view of the high iron content—not at all suitable for mainsprings. In fact such an alloy may be used for hairsprings having a constant and very small thermoelastic coefficient ranging in the neighbourhood of zero. Also the modulus of elasticity of such alloys ranges between 18,000 and 20,000 kg./mm.<sup>2</sup>. Moreover, springs made from such an alloy are relatively soft and show a limit of elasticity of about 80 kg./mm.<sup>2</sup>. Nevertheless such alloys are well suited for hairsprings, that is to say for springs which are not subjected to very strong strain.

In view of my experiences in the watch field and as a result of the many tests made over a period of many years with watch springs I have found that—in this art—even slight changes in the constitution of an alloy may cause important changes in the physical properties.

I have also found that—for the production of special alloy watch main springs requiring a very high modulus of elasticity—it is necessary that the alloy used therefor does not contain more than 25% of iron and should also comprise calculated small amounts of both beryllium and titanium.

The main object is thus a corrosion-resistant, substantially non-magnetic highly elastic main spring for watches constructed of an alloy of the following composition:

50 to 68% nickel

10 to 25% iron

10 to 25% chromium

A total of 5 to 10% of at least one metal of the group consisting of molybdenum and tungsten

0.005 to 1.2% beryllium

0.01 to 2% titanium, and

0 to 3% of manganese and silicon

In addition such an alloy may contain small quantities of conventional additives.

## 2

Indeed, the percentage of the various elements which constitute the new alloys vary within the ranges given above.

I have observed by experiments that main springs made of an alloy of the above composition are highly resistant to corrosion and show a modulus of elasticity ranging from 21,000 to 24,000, a value which never could be reached with springs made of an alloy as disclosed in my U. S. Patent No. 2,072,489, since the latter are too brittle. Moreover, main springs according to the present invention possess a limit of elasticity of about 160 kg./mm.<sup>2</sup>.

The following examples illustrate the invention, without however being limitative thereof.

|    | Example 1        | Percent |
|----|------------------|---------|
| 15 | Nickel -----     | 59      |
|    | Iron -----       | 15      |
|    | Chromium -----   | 15      |
| 20 | Molybdenum ----- | 7       |
|    | Beryllium -----  | 0.75    |
|    | Titanium -----   | 1       |

|    | Example 2        | Percent |
|----|------------------|---------|
| 25 | Nickel -----     | 59      |
|    | Iron -----       | 16      |
|    | Chromium -----   | 15.6    |
|    | Molybdenum ----- | 8       |
| 30 | Beryllium -----  | 0.3     |
|    | Titanium -----   | 0.8     |

|    | Example 3       | Percent |
|----|-----------------|---------|
| 35 | Nickel -----    | 59      |
|    | Iron -----      | 15      |
|    | Chromium -----  | 15      |
|    | Tungsten -----  | 7       |
| 40 | Beryllium ----- | 0.75    |
|    | Titanium -----  | 1       |

|    | Example 4       | Percent |
|----|-----------------|---------|
| 45 | Nickel -----    | 59      |
|    | Iron -----      | 16      |
|    | Chromium -----  | 15.6    |
|    | Tungsten -----  | 8       |
|    | Beryllium ----- | 0.3     |
| 50 | Titanium -----  | 0.8     |

|    | Example 5        | Percent |
|----|------------------|---------|
| 55 | Nickel -----     | 59      |
|    | Iron -----       | 16      |
|    | Chromium -----   | 16      |
|    | Tungsten -----   | 4       |
|    | Molybdenum ----- | 3       |
|    | Beryllium -----  | 0.75    |
|    | Titanium -----   | 1       |

|    | Example 6        | Percent |
|----|------------------|---------|
| 60 | Nickel -----     | 56      |
|    | Iron -----       | 24      |
|    | Chromium -----   | 11      |
|    | Tungsten -----   | 4       |
|    | Molybdenum ----- | 4       |
|    | Beryllium -----  | 0.01    |
|    | Titanium -----   | 0.05    |

|    | Example 7        | Percent |
|----|------------------|---------|
| 65 | Nickel -----     | 50      |
|    | Iron -----       | 18      |
|    | Chromium -----   | 21.2    |
|    | Tungsten -----   | 5       |
| 70 | Molybdenum ----- | 3       |
|    | Beryllium -----  | 1.1     |
|    | Titanium -----   | 1       |

## Example 8

|            | Percent |
|------------|---------|
| Nickel     | 65      |
| Iron       | 10      |
| Chromium   | 17      |
| Tungsten   | 4       |
| Molybdenum | 2       |
| Beryllium  | 1       |
| Titanium   | 0.8     |

## Example 9

|            |      |
|------------|------|
| Nickel     | 56.6 |
| Iron       | 15   |
| Chromium   | 21   |
| Tungsten   | 2    |
| Molybdenum | 4    |
| Beryllium  | 0.6  |
| Titanium   | 0.6  |

## Example 10

|            |      |
|------------|------|
| Nickel     | 56   |
| Iron       | 16   |
| Chromium   | 21.3 |
| Tungsten   | 2    |
| Molybdenum | 4    |
| Beryllium  | 0.2  |
| Titanium   | 0.3  |

## Example 11

|            |     |
|------------|-----|
| Nickel     | 51  |
| Iron       | 13  |
| Chromium   | 22  |
| Tungsten   | 4   |
| Molybdenum | 6   |
| Beryllium  | 0.9 |
| Titanium   | 1.5 |

## Example 12

|            |     |
|------------|-----|
| Nickel     | 50  |
| Iron       | 18  |
| Chromium   | 40  |
| Molybdenum | 21  |
| Beryllium  | 8   |
| Titanium   | 1.1 |

## Example 13

|            |     |
|------------|-----|
| Nickel     | 65  |
| Iron       | 11  |
| Chromium   | 15  |
| Molybdenum | 7   |
| Beryllium  | 1   |
| Titanium   | 0.8 |

## Example 14

|            |      |
|------------|------|
| Nickel     | 55   |
| Iron       | 15   |
| Chromium   | 22.7 |
| Molybdenum | 6    |
| Beryllium  | 0.6  |
| Titanium   | 0.6  |

## Example 15

|            |     |
|------------|-----|
| Nickel     | 56  |
| Iron       | 14  |
| Chromium   | 23  |
| Molybdenum | 6.3 |
| Beryllium  | 0.3 |
| Titanium   | 0.3 |

## Example 16

|           |      |
|-----------|------|
| Nickel    | 51   |
| Iron      | 16   |
| Chromium  | 20.5 |
| Tungsten  | 10   |
| Beryllium | 0.9  |
| Titanium  | 1.5  |

## Example 17

|           | Percent |
|-----------|---------|
| Nickel    | 51      |
| Iron      | 17      |
| Chromium  | 21      |
| Tungsten  | 10      |
| Beryllium | 0.25    |
| Titanium  | 0.5     |

## Example 18

|            |      |
|------------|------|
| Nickel     | 65   |
| Iron       | 16   |
| Chromium   | 10   |
| Tungsten   | 4.2  |
| Molybdenum | 4.3  |
| Beryllium  | 0.15 |
| Titanium   | 0.3  |

The percentages, in the preceding examples as well as in the following explanations, are throughout percentages by weight.

The alloys set forth in the examples may also contain small quantities of conventional deoxidizing agents and working-up additions, such for example as silicon and/or manganese, the total amount of these deoxidizers containing at least one of the metals selected from the group consisting of manganese and silicon ranging between 1 and 2%, although lesser or greater amounts may if desired be used.

Titanium-free alloys are known, the composition of which is otherwise the same as or similar to that of the alloys according to the present invention, and it has heretofore been the opinion of the skilled in the art that hardness, elasticity and resistance to corrosion of such known alloys could not be exceeded.

On the other hand, iron-free high nickel-containing alloys, having a small chromium and molybdenum content, and also containing beryllium and titanium, are known and these have been intended for use as springs.

However, none of these known alloys fulfills all the high requirements necessary, more especially, for mainsprings of clock and watch mechanisms.

Tests carried out for example with alloys of the following composition:

## Alloy No. 1 consisting of:

|                                                                                       |
|---------------------------------------------------------------------------------------|
| 15% iron                                                                              |
| 15% chromium                                                                          |
| 7% molybdenum                                                                         |
| 0.75% beryllium                                                                       |
| Remainder essentially nickel together with small quantities of silicon and manganese, |

on the one hand, and

## Alloy No. 2 consisting of:

|                 |
|-----------------|
| 15% iron        |
| 15% chromium    |
| 7% molybdenum   |
| 0.75% beryllium |
| 1% titanium     |

Remainder essentially nickel together with small quantities of silicon and manganese,

on the other hand, show that, while the two alloys have comparable hardness and rebound properties, i. e. capacity to return to original state after being flexed, the springiness in the case of alloy No. 2 is surprisingly greater than that of alloy No. 1. Other alloys of more or less similar composition and which have heretofore been proposed for the same purpose as the alloys of the present invention are even more inferior in this regard.

The provision, according to the present invention, of a content of beryllium and titanium in alloys of the type here involved, thus constitutes a considerable step forward in the art, the realized superiority being of especial importance when the alloys are used in mainsprings of clocks and watches.

Having thus disclosed the invention, what is claimed is:

1. A corrosion-resistant, substantially non-magnetic highly elastic mainspring for watches constructed of an alloy of the following composition:

59% nickel  
15% iron  
15% chromium  
7% molybdenum  
0.75% beryllium  
1% titanium and

The remainder being at least one metal of the group consisting of manganese and silicon.

2. A corrosion-resistant, substantially non-magnetic highly elastic mainspring for watches constructed of an alloy of the following composition:

59% nickel  
15% iron  
15% chromium  
7% tungsten  
0.75% beryllium  
1% titanium and

The remainder being at least one metal of the group consisting of manganese and silicon.

3. A corrosion-resistant, substantially non-magnetic highly elastic mainspring for watches constructed of an alloy of the following composition:

59% nickel  
15% iron  
12% chromium  
5 to 10% of at least one metal of the group consisting of molybdenum and tungsten  
0.75% beryllium  
1% titanium and

The remainder being at least one metal of the group consisting of manganese and silicon.

4. A corrosion-resistant, substantially non-magnetic highly elastic mainspring for watches constructed of an alloy of the following composition:

59% nickel  
16% iron  
15.6% chromium  
8% tungsten  
0.3% beryllium  
0.8% titanium

The remainder being at least one metal of the group consisting of manganese and silicon.

5. A corrosion-resistant, substantially non-magnetic

highly elastic mainspring for watches constructed of an alloy of the following composition:

59% nickel  
16% iron  
16% chromium  
4% tungsten  
3% molybdenum  
0.75% beryllium  
1% titanium and  
10 The remainder being at least one metal of the group consisting of manganese and silicon.

6. A corrosion-resistant, substantially non-magnetic highly elastic mainspring for watches constructed of an alloy of the following composition:

56% nickel  
16% iron  
21.3% chromium  
2% tungsten  
20 4% molybdenum  
0.2% beryllium  
0.3% titanium  
The remainder being at least one metal of the group consisting of manganese and silicon.

25 7. A corrosion-resistant, substantially non-magnetic highly elastic mainspring for watches constructed of an alloy having the following composition:

55-59% nickel  
30 14-16% iron  
12-22.7% chromium  
5-10% of at least one metal selected from the group consisting of molybdenum and tungsten  
0.2-1.2% beryllium  
35 0.3-2% titanium  
The remainder being at least one metal of the group consisting of manganese and silicon, the total of Mn+Si being not in excess of 3%.

#### References Cited in the file of this patent

##### UNITED STATES PATENTS

|              |               |       |               |
|--------------|---------------|-------|---------------|
| 1,942,150    | Rohn          | ----- | Jan. 2, 1934  |
| 2,072,489    | Straumann     | ----- | Mar. 2, 1937  |
| 45 2,090,044 | Hessenbruch   | ----- | Aug. 17, 1937 |
| 2,164,951    | Schwartz      | ----- | July 4, 1939  |
| 2,524,661    | Harder et al. | ----- | Oct. 3, 1950  |

##### FOREIGN PATENTS

|            |               |       |                |
|------------|---------------|-------|----------------|
| 50 263,074 | Switzerland   | ----- | Aug. 15, 1949  |
| 585,151    | Germany       | ----- | Sept. 29, 1933 |
| 608,297    | Germany       | ----- | Jan. 19, 1935  |
| 583,845    | Great Britain | ----- | Jan. 1, 1947   |